

Nov. 6, 1934.

P. KÜHN

1,979,629

STEEL AND PROCESS FOR ITS PRODUCTION

Filed Aug. 29, 1930

4 Sheets-Sheet 1

Variation of The Chemical Composition  
of Steel and Slag During THE Melting Process

Melt A



Melt B



C — Mn — FeO — MnO — CaO

Inventor:  
P. Kuhn

By: Marks Heiss  
1934

Nov. 6, 1934.

P. KÜHN

1,979,629

STEEL AND PROCESS FOR ITS PRODUCTION

Filed Aug. 29, 1930

4 Sheets-Sheet 2

TENACITY PROPERTIES OF STEELS ACCORDING TO THE SPECIAL DEOXIDIZING PROCESS.  
32 RESULTS OF TESTING  
SHEETS OF 15 TO 30 MM  
THICKNESS.



TENACITY PROPERTIES OF ORDINARY CARBON STEELS



Inventor:  
P. Kuhn

By: Marks & Clark  
Attest.

Nov. 6, 1934.

P. KÜHN

1,979,629

STEEL AND PROCESS FOR ITS PRODUCTION

Filed Aug. 29, 1930

4 Sheets-Sheet 3

NOTCH TENACITY BEFORE AND AFTER AGING TREATMENT DEPENDANT  
ON THE TESTING TEMPERATURE 20 MM SHEET FROM MELT-A



— ANNEALED AT 900°C, 1 HOUR AIR COOLING.  
— ANNEALED AT 900°C, 1 HOUR AIR COOLING.  
— 10% UPSET ACID TEMPERED.

STANDARD 20 MM BOILER PLATE



— ANNEALED AT 900°C, 1 HOUR  
— ANNEALED AT 900°C, 1 HOUR AIR COOLING,  
10% UPSET ACID TEMPERED.

Inventor:  
P. Kuhn

By: Marks & Elvey  
Attest.

Nov. 6, 1934.

P. KÜHN

1,979,629

STEEL AND PROCESS FOR ITS PRODUCTION

Filed Aug. 29, 1930

4 Sheets-Sheet 4

NOTCH TENACITY BEFORE AND AFTER THE AGING  
TREATMENT DEPENDENT ON THE TESTING TEMPERATURE.  
20 mm PLATE FROM MELT B.



Inventor:

P. Kuhn

By: Marks & Elan  
Atty's.

## UNITED STATES PATENT OFFICE

1,979,629

## STEEL AND PROCESS FOR ITS PRODUCTION

Paul Kühn, Niederschelden-on-the-Sieg, Germany, assignor to Vereinigte Stahlwerke Aktiengesellschaft, Dusseldorf, Germany

Application August 29, 1930, Serial No. 478,749  
In Germany September 14, 1929

5 Claims. (Cl. 75—27)

This invention relates to a process for obtaining steel of high tenacity and low sensitivity to cold shortness, ageing, and brittleness at blue heat in basic open hearth furnaces.

5 Considered from the point of view of the chemical reactions taking place in the bath or melt, basic open hearth smelting processes are auto oxidation processes. The foreign constituents in the melt are oxidized depending upon their affinity for oxygen and to an extent determined by the concentration and temperature and pass into the slag or into the waste gases. As the concentration of reducing substances in the bath decreases the iron also is oxidized to ferrous and ferric oxide 10 to an increasing extent, especially towards the end of the smelting operation. Inasmuch as ferric oxide ( $Fe_2O_3$ ) is unstable in the presence of metallic iron and of the reducing substances present in the bath at the high temperatures obtaining in the smelting furnace the bulk of the oxidized iron consists of ferrous oxide (FeO). Ferrous oxide is soluble to a certain extent in the slag and also in the molten metal, the degree of distribution of same in the slag and in the bath being determined by the Nernst partition co-efficient. The concentration of ferrous oxide in the bath has therefore a certain direct relationship to that in the slag and it is therefore possible to draw comparative conclusions from the concentration of the 15 metallic oxide in the slag, as to the extent to which the metallic oxides have dissolved in the bath.

The fundamental reason for the continuous progress of the fining operation in basic open hearth furnaces is according to Mars probably to be attributed to the fact that the constructional materials of the furnace and the slag-forming constituents of the basic open hearth furnace, i. e. magnesia and lime cannot enter into chemical 20 combination with the ferrous oxide of the bath, but can only form physical solutions with the metallic oxides, so that the reactive power of the dissolved ferrous oxide with the carbon in the bath remains unaffected, and the boiling-up and fining operations therefore proceed continuously. As the concentration of reducing substances in the bath decreases the ferrous oxide content of the slag and also that of the bath increases rapidly 25 towards the end of the smelting process on account of the oxidizing action of the gases. As is known, test bars of steel, taken from the bath at this period usually exhibit red shortness on bending at a red heat to a greater or lesser degree.

Dichmann, a well-known authority on the operation of basic open hearth furnaces, considers

that a state of equilibrium with respect to the ferrous oxide content in the slag and the reducing substances in the iron is reached for all practical purposes when the ferrous oxide content of the slag has been reduced to 13% FeO (corresponding to 10% Fe). At the same time the slag also contains about the same quantity of MnO. As is taught by practical experience however, it is not always possible in the ordinary course of working to produce steel having a low carbon content 60 underneath a slag containing only 10% of iron without undue difficulty; usually the iron content of the slag is somewhat higher.

When the desired carbon content has been obtained the fining process must be brought to 70 a finish—forcibly to a certain extent—by the addition of deoxidizing agents. As is known the chief problem of deoxidizing is to remove the residual oxygen which exists in a state of equilibrium in the bath with carbon. The deoxidizing 75 agents chosen—apart from carbon which is only used in exceptional cases—are ferrous alloys, the metallic constituents of which on account of their great affinity for oxygen as compared with that possessed by iron, are able to remove said 80 oxygen. All the deoxidizing agents with the exception of carbon, form solid or liquid products which are partly retained in the iron in a finely divided heterogeneous condition throughout the solidification period and constitute a portion of 85 the known non-metallic constituents of the steel. These constituents reduce the technical properties of the steel as is known and lead to the production of longitudinal cracks and sensitivity on 90 hardening and when the steel is subjected to varying stresses they are usually the starting points for fatigue fracture. For this reason according to Eilender deoxidation with agents which produce solid deoxidation products, should be avoided as far as possible.

95 A further drawback of the usual deoxidation processes towards the end of the smelting operation is the fact that when employing ferro-manganese for example it is impossible completely to remove the oxygen even when using large quantities of the deoxidation agent, for invariably only a definite state of equilibrium can be reached. Experiments have therefore been carried out using gradual deoxidation with metals which exhibit a progressively increasing affinity for oxygen, and it is possible in this manner by adding large quantities of aluminium for example, to produce steel with a very small content of oxygen. The disadvantages of this deoxidizing process 100 still persists however, because the oxidation 105

110

product of aluminium, i. e. alumina is retained very readily by steel in a finely dispersed condition after the manner of an emulsion.

If the foregoing statements be considered as a whole, basic open hearth smelting processes can be looked upon as processes with automatic oxidation of the molten metal bath and induced indirect deoxidation by the addition of ferrous alloys, whereby solid or liquid oxidation products are usually formed which are readily retained by the steel. On the other hand according to Mars the crucible smelting process and in a similar manner the acid open hearth process form after the completion of the fining process, typical examples of a process with automatic deoxidation. During the acid process when definite conditions are maintained the last traces of oxygen in the steel existing as FeO form a stable chemical compound of iron silicate with the silica of the lining which passes into the slag. At the same time owing to the action of the pure iron, silicon is reduced from the lining and this silicon takes up the remaining traces of oxygen. According to Mars, the excellent properties of acid steel can be attributed partly to this automatic deoxidation by virtue of which only very small quantities of impurity or even no impurities at all are retained by the steel.

The present process occupies an intermediate position between the acid and the basic open hearth smelting processes, inasmuch as it forcibly effects in the basic process a certain automatic deoxidation during the whole smelting process by means of manganese in a similar manner to the role of the silicon in the acid furnace. The important part played by the manganese during the control of the desulphurizing process and the usual deoxidation shortly before tapping is known per se. It is also known to add large quantities of manganese to the charge when it is desired to smelt a high value steel. However when producing soft steel in the basic open hearth furnace the percentage of manganese in the charge is kept as far as is possible below 1.5% inasmuch as killing has shown that the exploitation of manganese and consequent thereupon the economy of the process are reduced very considerably upon still further increasing the manganese content.

According to the process of the present invention this rule is deliberately disregarded and large quantities of oxygen are prevented from combining with the steel even during the smelting process—which is to be carried out as rapidly as possible in view of the oxidation—by means of a large charge of manganese, since the manganese is first converted into slag to a preponderant extent. After the melt has been run down completely, when the charge has been com-

pletely transformed into the molten state and the bulk of the manganese has been oxidized and transformed into the slag, large amounts of lime are added according as the temperature rises above the usual level, thus setting free metallic oxides from compounds in the slag and effecting the reduction by the reducing substances in the bath. The quantity of lime added varies naturally according to the amount of the acids in the slag to be combined; under the working conditions of the present case the amount of lime to be added varies between 1-2% (this amount increasing with rising furnace temperatures) of the amount of the charge. After the lime has been added the temperature is further raised as rapidly as possible and the slag is kept as mobile as possible in order to increase the velocity of reaction in the reaction zone between the slag and the bath and also to increase the absorptive capacity of the slag for further amounts of lime. Since the ferrous oxide content of the slag is already relatively low on running down, whilst moreover the slag contains large quantities of MnO, about 30-40%, this amount being lower at specially high temperatures, the MnO is vigorously reduced from out of the slag and the manganese is transferred to the bath. The reduced manganese in *statu nascendi* reduces the ferrous oxide dissolved in the steel very vigorously, the ferrous oxide content of the slag being also continuously reduced at the same time. The MnO formed by this reaction is again reduced in a cycle by the carbon content of the bath until finally the ferrous oxide content of the slag and bath has been reduced to an extremely small amount. The manganese content of the bath increases considerably in parallel to this automatic deoxidation by means of the manganese reduced from out of the slag—in many cases up to 1.3% of manganese and over. Operating with a highly basic slag naturally requires an elevated and uniform temperature throughout the whole smelting operation, which may be assured for example by using the regenerative furnaces described in Patent 1,421,259.

When the desired concentration of carbon has been reached the melt is tapped off without the usual deoxidation process, i. e. in general without any further additions. Additions of any desired alloy constituents can obviously be made in the usual manner either in the furnace, during the tapping off in the trough or in the pan. On account of the lack of any perceptible amount of oxygen the steel solidifies very quietly as the reaction:



which gives rise to the formation of gas, cannot occur.

60

TABLE 1

13

Chemical composition of preliminary test portions of steel and slag taken from melt A

| Constituent | 1     | 2     | 3     | 4     | 5     | 6     | 7     | 8     | 9     | 10    | 11    | 12    | 13    | 14 |
|-------------|-------|-------|-------|-------|-------|-------|-------|-------|-------|-------|-------|-------|-------|----|
| Metal       | 0.76  | 0.67  | 0.60  | 0.56  | 0.47  | 0.42  | 0.40  | 0.37  | 0.33  | 0.26  | 0.24  | 0.20  | 0.15  |    |
|             | 0.48  | 0.50  | 0.61  | 0.70  | 0.81  | 0.83  | 0.90  | 0.84  | 0.82  | 0.81  | 0.75  | 0.74  | 0.76  |    |
|             | 0.058 | 0.061 | 0.058 | 0.049 | 0.043 | 0.037 | 0.036 | 0.032 | 0.031 | 0.027 | 0.029 | 0.026 | 0.022 |    |
|             | 0.047 | 0.046 | 0.044 | 0.046 | 0.044 | 0.038 | 0.034 | 0.036 | 0.034 | 0.032 | 0.034 | 0.032 | 0.030 |    |
| Slag        | 16.46 | 16.42 | 15.00 | 16.00 | 16.16 | 15.06 | 14.28 | 14.00 | 13.90 | 13.00 | 13.25 | 12.50 | 12.80 |    |
|             | 0.73  | 0.64  | 0.71  | 0.94  | 1.47  | 1.33  | 1.58  | 1.45  | 1.37  | 1.51  | 1.58  | 1.42  | 1.40  | 14 |
|             | 15.73 | 15.05 | 9.25  | 13.20 | 9.12  | 6.60  | 8.19  | 5.68  | 7.53  | 10.04 | 10.04 | 5.42  | 7.92  |    |
|             | 1.90  | 2.20  | 11.26 | 1.59  | 1.87  | 6.56  | 2.79  | 8.35  | 8.79  | 2.05  | 2.78  | 11.99 | 9.36  |    |
|             | 1.06  | 0.55  | 0.40  | 0.60  | 0.86  | 1.25  | 1.49  | 1.28  | 0.92  | 1.00  | 1.12  | 0.80  | 0.70  |    |
|             | 17.88 | 17.88 | 20.05 | 27.02 | 37.11 | 37.47 | 39.47 | 39.71 | 40.30 | 43.18 | 43.30 | 39.73 | 39.89 |    |
|             | 5.96  | 6.55  | 6.63  | 6.00  | 6.43  | 6.32  | 6.80  | 6.58  | 6.78  | 6.26  | 7.61  | 7.61  | 7.61  |    |
| 75          | 39.60 | 39.85 | 36.24 | 34.14 | 26.59 | 25.00 | 24.71 | 22.33 | 19.80 | 21.56 | 21.00 | 20.00 | 19.81 |    |
|             | 0.11  | 0.16  | 0.07  | 0.13  | 0.30  | 0.08  | 0.16  | 0.10  | 0.15  | 0.37  | 0.37  | 0.19  | 0.23  |    |

TABLE 2

Chemical composition of preliminary test portions of steel and slag taken from melt B

| 5     | Constituent                    | 1     | 2     | 3     | 4     | 5     | 6     | 7     | 8     | 9     | 10    | 11    | 80 |
|-------|--------------------------------|-------|-------|-------|-------|-------|-------|-------|-------|-------|-------|-------|----|
| Metal | C                              | 0,87  | 0,80  | 0,72  | 0,67  | 0,62  | 0,56  | 0,52  | 0,47  | 0,43  | 0,37  | 0,32  |    |
|       | Mn                             | 0,54  | 0,49  | 0,57  | 0,65  | 0,74  | 0,77  | 0,85  | 0,86  | 0,88  | 0,89  | 0,92  |    |
|       | P                              | 0,041 | 0,037 | 0,039 | 0,039 | 0,037 | 0,037 | 0,039 | 0,034 | 0,041 | 0,032 | 0,043 |    |
|       | S                              | 0,046 | 0,047 | 0,043 | 0,050 | 0,048 | 0,048 | 0,052 | 0,046 | 0,049 | 0,042 | 0,036 |    |
| 10    | SiO <sub>2</sub>               | 19,90 | 19,05 | 19,80 | 18,90 | 17,80 | 18,20 | 19,30 | 19,34 | 18,20 | 17,45 | 16,30 |    |
|       | CaO                            | 0,32  | 0,18  | 0,32  | 0,23  | 0,64  | 0,59  | 0,72  | 0,73  | 0,72  | 0,73  | 0,78  |    |
|       | FeO                            | 11,56 | 11,69 | 11,63 | 10,10 | 10,26 | 10,31 | 8,84  | 8,98  | 8,98  | 8,46  | 8,86  |    |
|       | Fe <sub>2</sub> O <sub>3</sub> | 2,26  | 1,69  | 1,14  | 1,14  | 0,74  | 1,46  | 1,02  | 0,73  | 0,73  | 1,59  | 3,42  |    |
| Slag  | Al <sub>2</sub> O <sub>3</sub> | 2,43  | 2,50  | 2,00  | 2,13  | 1,85  | 1,32  | 1,53  | 0,71  | 0,65  | 1,61  | 1,37  |    |
|       | CaO                            | 15,22 | 18,09 | 22,41 | 30,12 | 28,70 | 29,50 | 33,40 | 35,27 | 35,80 | 37,49 | 36,16 |    |
|       | MgO                            | 0,00  | 9,99  | 9,06  | 8,41  | 9,80  | 9,10  | 9,12  | 8,75  | 9,00  | 9,51  | 10,02 |    |
|       | MnO                            | 38,12 | 36,16 | 33,64 | 28,78 | 29,57 | 28,47 | 25,72 | 24,55 | 24,32 | 22,74 | 22,51 |    |
| 15    | S                              | 0,10  | 0,11  | 0,14  | 0,11  | 0,20  | 0,22  | 0,23  | 0,26  | 0,26  | 0,26  | 0,21  |    |

Tables 1 and 2 give as examples of the herein-before described process, analyses taken every 15 minutes of test portions of steel and slag taken from the furnace, Table 1 being for a soft metal (A) and Table 2 being for a melt B of medium hardness. The charge consisted in both cases of about 25% of steel-iron containing 4 to 5% of manganese, 30% of soft scrap core iron, the remainder being sheet scrap. The course of the variation in the amounts of the most important constituents such as carbon and manganese in the case of the steel, and MnO, CaO, and FeO in the case of the slag is illustrated in the case of melt A in Figure 1, and in the case of melt B in Figure 2.

Figs. 1 and 2 respectively show in melts A and B the variation of the chemical composition of steel and slag during the melting process;

Fig. 3 shows the tenacity properties of steels produced according to the special deoxidizing process;

Fig. 4 shows tenacity properties of ordinary carbon steel;

Fig. 5 shows notch tenacity of 20 mm. steel from melt A;

Fig. 6 shows notch tenacity of standard 20 mm. boiler plate;

Figs. 7 and 8 show notch tenacity of 20 mm. plate from melt B and standard steel 48-22 mm. diameter, respectively.

In Figures 1 and 2 the two series of ordinates represent the percentage of carbon and manganese in the steel and the percentage of FeO, MnO and CaO in the slag respectively, whilst the abscissæ represent the numbers of the test-pieces.

Melt A was run down with a carbon content of 0.76%. Soon after it had been run down considerable quantities of lime and some fluor-spar were added at short intervals. As the lime content of the slag increased and the temperature rose and the carbon content decreased, an extremely violent reduction of MnO in the slag took place. As the concentration of MnO decreased the concentration of manganese in the steel increased until test No. 7 showed a concentration of 0.90%. Concomitant with the reduction of manganese, deoxidation which was not quite uniform took place, and the FeO content in the slag was reduced until on tapping it was about 8%. As the carbon content was reduced still further the deoxidation took place towards the end of the fusion partly at the expense of the manganese content in the bath, as was indicated by the decrease in concentration of manganese. The preliminary steel test bars were completely free from red shortness even after being run-down and could be hammered down thoroughly during the notched-bar test as from test piece No. 7.

Melt B (Table 2 and Figure 2) was somewhat more difficult to run down than melt A. After the first test portion had been taken 500 kilogrammes of lime were added in consequence of which the CaO content rose rapidly to 30%. After tests 5-9 100 kgs. of lime were added each time, whereupon the CaO content increased to about 40%, the temperature rising at the same time. From test 2 onwards vigorous reductions of the manganese from the slag took place. The MnO content of the slag was reduced to 23%, the FeO content was already very low after running down and during the course of the smelting operation it sank apparently uniformly to about 8% on tapping. The red shortness tests and notched bar impact tests carried out during the course of the smelting process were satisfactory. The steel solidified absolutely quietly.

The automatic deoxidation can therefore be considered as being complete, when the FeO content of the slag prior to tapping is at the maximum 10%, whilst the manganese content of the steel is rising uniformly. No limitation at all exists with respect to the carbon content in the final product as is shown from the attached documents. The process is applicable with the same security and advantage to the production of soft and medium hard or hard steel whether it be unalloyed or alloyed.

The technical properties of steel produced in accordance with the present invention are characterized essentially by a high elongation and notched bar tenacity in comparison with the tensile strength. These steels are at the same time practically insensitive to stresses due to ageing, working at a blue heat and other harsh treatment in working routine. Figure 3 gives the mean values for the results of numerous tensile strength tests on the products produced by the present process. Figure 4 gives tensile strength properties of the ordinary open hearth steel.

In these figures tensile strength and elastic limit in kgs. per mm<sup>2</sup> and elongation and reduction of area as percentages are plotted against the percentage of carbon contained in the steel.

As can be recognized from Figure 3 the values for the elongation and the notched bar tenacity are greater than those of the ordinary carbon steels particularly in the case of steels of medium hardness. In the case of the elongation the increase amounts to about 5 units, whilst the notched bar tenacity is about 100% greater. The steels were tested in the normalized condition.

As is known the sensitivity to ageing is specially influenced by the concentration of oxygen dissolved in the iron. The steels manufactured by the present process are in practice very deficient in respect of the sensitivity to ageing.

Since as is known the effect of ageing treatment consists substantially in a displacement of the steep drop in the notched bar tenacity-temperature curve in a direction of higher temperatures, the gauging of the ageing effect produced at normal temperatures is facilitated by examining the notched bar tenacity of the steel prior to and subsequent to ageing treatment at elevated and at low temperatures. In the ageing tests carried out by the applicant the test pieces having dimensions of 10x11x60 mm. were upset by means of a stamp to the extent of about 10%, were annealed for one hour at 250° C., and were subsequently subjected to notched bar tenacity tests and were examined at temperatures ranging from -80° to 200° C. The dimensions of the test pieces were then 10x10x60 mm. each having a semicircular notch 5 mm. in depth and 2 mm. across. In Figure 5 the results of notched bar ageing tests carried out upon test pieces taken from the centre of a 20 mm. sheet from melt A are given in dependency upon the testing temperature. Figure 6 contains the results of tests carried out under similar conditions upon ordinary boiler sheet metal of the same tensile strength. Similarly in Figures 7 and 8 results of notched bar tests carried out on a heat-treated 20 mm. sheet taken from melt B and by way of comparison results upon a 22 mm. cylindrical rod made of ordinary open hearth steel of the same tensile strength are given.

In Figures 5, 6, 7, and 8 the notched-bar tenacity in mkg. per sq. cm. before and after ageing treatment is plotted against the testing temperature. The full line gives the result when the test-bar is subjected to heat treatment at 900° C. for one hour, and is cooled in the air. The thin line gives the result when the test-bar is subjected to heat-treatment for one hour at 900° C., is cooled in the air, is upset to the extent of 10% and annealed.

As is shown in Figure 5 the steep drop of the curve prior to the ageing treatment begins at -20° C.; at -50° C. the sheet steel still has a notched-bar tenacity of 6 mkg. per sq. cm.

The steep drop of the curve is displaced by virtue of the ageing treatment by about 30° in the direction of more elevated temperatures, the fall begins at 0° C. and is consequently not yet perceptible at room temperature. The notched bar tenacity at room temperature is thus merely lowered from 11.4 down to 10.9 mkg. per sq. cm. by the ageing treatment. The sheet metal is substantially insensitive to ageing. Figure 6 shows results of tests carried out on ordinary boiler sheet metal. In the unaged condition the steep drop begins at room temperature. By virtue of the ageing treatment such drop is displaced by almost 100° in the direction of more elevated temperatures with the result that the sheet metal up to testing temperatures of 50° C. is brittle. The notched bar tenacity at room temperature has thus been lowered from 11 down to about 1 mkg. per sq. cm. In the case of melt B the notched bar tenacity at room temperature is reduced by the ageing treatment from 9 to 8.2 mkg. per sq. cm. and in the case of ordinary carbon steel from 8.5 to 2.5 mkg. per sq. cm., i. e. a substantially greater reduction.

Steels produced in accordance with the present invention are for practical purposes free from segregation phenomena and have a very low oxygen content. It has been shown as the result of exhaustive experiments that they have an ex-

tremely high resistance to the action of overheating, recrystallization and fusion welding, which tend to increase the size of the grain.

I claim:

1. A two-period process of producing a steel 80 of high tenacity and low sensitivity to cold brittleness, ageing and blue shortness in a basic open hearth furnace, which comprises oxidizing manganese during the first of said periods and transferring said manganese into the slag and 85 then continuously reducing manganese from the slag and continuously increasing the manganese content of the steel throughout the second period, thereby transferring the reduced manganese from the slag into the bath so that the process is terminated without adding ferro-manganese as a deoxidizing agent before the tapping. 90

2. A process of producing steel of high tenacity and low sensitivity to cold brittleness, ageing and blue shortness in a basic open hearth furnace, consisting in transferring manganese into the slag during an oxidation period, raising the temperature and adding basic materials to reverse the transformation of the manganese, thereby continuously reducing and transferring 100 manganese from the slag into the bath during the entire period calculated from the reversal of the transformation to the tapping so that the process is terminated without adding ferro-manganese as a deoxidizing agent before the tapping. 105

3. A process of producing a steel of high tenacity and low sensitivity to cold brittleness, ageing and blue shortness in a basic open hearth furnace, consisting in transferring manganese into the slag during an oxidation period, raising 110 the temperature and adding lime to reverse the transformation of the manganese, thereby continuously reducing and transferring manganese from the slag into the bath during the entire period calculated from the reversal of the transformation to the tapping so that the process is terminated without adding ferro-manganese as a deoxidizing agent before the tapping. 115

4. A process of producing a steel of high tenacity and low sensitivity to cold brittleness, 120 ageing and blue shortness in a basic open hearth furnace, consisting in transferring the bulk of the manganese contained in the bath into the slag during the oxidation process, adding basic materials and continuing to raise the temperature, 125 thereby reversing the transformation of the manganese and continuously reducing and transferring manganese from the slag into the bath during the entire period calculated from the reversal of the transformation to the tapping so that the process is terminated without adding ferro-manganese as a deoxidizing agent before the tapping. 130

5. A process of producing a steel of high tenacity and low sensitivity to cold brittleness, 135 ageing and blue shortness in a basic open hearth furnace, consisting in transferring the bulk of the manganese contained in the bath into the slag during the oxidation process, adding lime and continuing to raise the temperature thereby reversing the transformation of the manganese and continuously reducing and transferring manganese from the slag into the bath during the entire period calculated from the reversal of the transformation to the tapping so that the process is 140 terminated without adding ferro-manganese as a deoxidizing agent before the tapping. 145

PAUL KÜHN.